

# United States Patent Office

2,875,050

Patented Feb. 24, 1959

1

2,875,050

## TRIAMINOPYRIDINE DEVELOPER

Gershon M. Goldberg, Arlington, and James E. Lu Valle, Lexington, Mass., assignors to Technical Operations Incorporated, Burlington, Mass., a corporation of Delaware

No Drawing. Application December 16, 1957  
Serial No. 702,759

9 Claims. (Cl. 96—66)

This invention relates to the art of photography and more particularly to the development of the latent silver image in exposed photographic emulsions.

The principal object of this invention is to provide improved photographic development with solutions which are more active than hydroquinone and which have a lower fog level than p-methylaminophenol ("Elon") or 1,2,4-benzenetriamine. A further object of this invention is to provide superadditive developing solutions which comprise new mixtures of active developing agents.

In a brief summary of this invention, these objects are achieved by the method of developing photographic film which comprises treating an exposed silver halide emulsion with a solution of 2,3,6-triaminopyridine. The developing solution preferably comprises 2,3,6-triaminopyridine, an anti-oxidant, an alkali and an anti-fogging agent dissolved in water and preferably has a pH between about 10 and 11. 1-phenyl-3-pyrazolidone ("Phenidone") added to the triaminopyridine developer solution greatly increases the speed of the solution while the addition of small amounts of triaminopyridine to conventional hydroquinone solutions forms a superadditive developer wherein the speed and maximum density are greatly increased and the gamma raised.

The following description illustrates developers according to this invention.

A typical developer solution according to the invention is as follows:

|                              |      |       |
|------------------------------|------|-------|
| Sodium carbonate -----       | g    | 42.4  |
| Sodium bromide -----         | g    | 2.0   |
| Sodium sulfite -----         | g    | 31.0  |
| 2,3,6-triaminopyridine ----- | mole | 0.025 |
| Water to make 2 liters.      |      |       |

In the above solution the active developing agent is the triaminopyridine while the carbonate, bromide and sulfite serve their usual function as an alkali, a restrainer or anti-fogging agent, and preservative or anti-oxidant respectively. Other alkali, anti-oxidant, and anti-fogging agents well known in the developer art can also be employed.

Strips of Plus X film of the Eastman Kodak Company were exposed through a standard step-wedge and developed in a standard Jarrell-Ash processing unit. The results of these tests are indicated in Table I below. In this table the 2,3,6-triaminopyridine is abbreviated TAP and was used in the formula disclosed above. The other tests indicated were also run with the same formula excepting that the particular developer indicated in each test was substituted for the triaminopyridine. In each of these tests an unexposed strip of the same film was processed alongside the exposed test strip as a control and to determine the fog level. The time of development was eight minutes and the temperature of the developer solutions was 68° F. After processing the densities were determined for each of the exposure steps and H and D curves were plotted. The speed was taken as the antilog (3-log E at D=0.2 above (fog+base).

2

Table I

| 5  | Developer                    | Molar conc. Developer | pH   | Fog | Speed | Gamma | Max. Dens. |
|----|------------------------------|-----------------------|------|-----|-------|-------|------------|
| 10 | TAP -----                    | .025                  | 10.5 | .27 | 20    | .75   | 1.39       |
|    | Hydroquinone -----           | .025                  | 10.5 | .28 | 8     | .61   | 1.00       |
|    | Phenidone -----              | .005                  | 10.5 | .29 | 20    | .39   | 1.00       |
|    | Elon -----                   | .025                  | 10.5 | .71 | 27    | 1.32  | 2.61       |
|    | 1,2,4-Benzene-triamine ----- | .025                  | 10.5 | .55 | 38    | .75   | 1.85       |

Table II below illustrates the development obtained by TAP alone and in combination with other common developing agents. The pH of each developing solution was 10.5 and the development time was eight minutes. The developing solutions contained the materials initially indicated except that the developers indicated in Table II replaced the triaminopyridine in the amounts stated. These data show that the combination of Phenidone and TAP produces an appreciable speed increase. With Elon, TAP appears to inhibit the developing activity of the Elon. When a small amount of hydroquinone is added to a TAP developer, the combination appears to produce only a small improvement. However, in TAP-hydroquinone combinations wherein the hydroquinone is the major molar ingredient, a superadditive developer appears to result. According to these data the speed and maximum density of hydroquinone are doubled and the gamma is raised.

Table II

| 35 | Test  | Developer              | Molar Conc. Developer | Fog | Speed | Gamma | Max. Dens. |
|----|-------|------------------------|-----------------------|-----|-------|-------|------------|
| 1  | ----- | TAP -----              | .025                  | .27 | 20    | .75   | 1.39       |
| 2  | ----- | TAP+Phenidone -----    | { .025<br>.005 }      | .31 | 63    | .62   | 1.57       |
| 3  | 40    | TAP+Hydroquinone ----- | { .030<br>.005 }      | .28 | 19    | 0.84  | 1.52       |
| 4  | ----- | TAP+Hydroquinone ----- | { .025<br>.006 }      | .30 | 19    | 1.05  | 2.00       |
| 5  | ----- | Hydroquinone -----     | .025                  | .28 | 8     | .61   | 1.00       |

Table III below indicates the development obtained with TAP developing solutions with various development times. TAP developing solutions of this concentration appear to have an induction period of about four minutes before development becomes evident. This induction period is not as long as that observed with hydroquinone since the same concentration of hydroquinone produces the first visible development in about eight minutes. Table III shows that TAP in this concentration produces adequate development in about eight minutes but that development for sixteen minutes is optimal. With the long developing times TAP becomes quite energetic and its action compares very favorably with other high energy developers.

Table III

[TAP development at 0.025 M and pH 10.5.]

| 60      | Time | Fog | Speed | Gamma |
|---------|------|-----|-------|-------|
| 1 min.  |      | 21  |       |       |
| 2 min.  |      | 21  |       |       |
| 4 min.  |      | 22  |       |       |
| 8 min.  |      | 25  | 3     | .23   |
| 16 min. |      | 37  | 15    | .67   |
| 32 min. |      | 38  | 63    | 1.11  |
|         |      |     | 102   | 1.24  |

Increasing the concentration of TAP from 0.025 to 0.050 M produces a large speed increase. Further increases in concentration produce relatively small effects. In the absence of bromide ion, the speed of development

increases from pH 9 to pH 11 and then falls off sharply at pH 12. In the presence of a moderate concentration of bromide ion (up to 0.02 M) TAP develops best at about pH 10. Higher pH's cause a sharp rise in the fog level. The presence of larger concentrations of bromide ions suppresses development with TAP developer solutions as well as with hydroquinone solutions up to about pH 10.5. The proper pH range for TAP developing solutions is thus about 10 to 11.

As illustrated by the foregoing data, tests indicate that TAP is similar to hydroquinone in its action and is generally a stronger developing agent. 2,3,6-triaminopyridine together with methods for its preparation are disclosed in United States Patent No. 2,136,044.

It should be understood that the foregoing disclosure is for the purpose of illustration only and that the invention includes all modifications falling within the scope of the appended claims.

We claim:

1. The method of developing photographic film which comprises treating an exposed silver halide emulsion with a solution of 2,3,6-triaminopyridine.
2. The method according to claim 1 wherein said solution has a pH between about 10 and 11.
3. The method of developing photographic film which comprises treating an exposed silver halide emulsion with

a solution of 2,3,6-triaminopyridine and 1-phenyl-3-pyrazolidone.

4. The method of developing photographic film which comprises treating an exposed silver halide emulsion with a solution of 2,3,6-triaminopyridine and hydroquinone.

5. A developing solution for exposed photographic silver halide emulsion which comprises 2,3,6-triaminopyridine, an anti-oxidant, an alkali, and an anti-fogging agent dissolved in water.

10 6. A developing solution according to claim 5 which has a pH between about 10 and 11.

7. A developing solution for exposed photographic silver halide emulsion which comprises 2,3,6-triaminopyridine, sodium sulfite, sodium carbonate, and sodium bromide dissolved in water, said solution having a pH between about 10 and 11.

8. A developing solution for exposed photographic silver halide emulsion which comprises 2,3,6-triaminopyridine and 1-phenyl-3-pyrazolidone dissolved in water.

15 9. A superadditive developing solution for exposed photographic silver halide emulsion which comprises 2,3,6-triaminopyridine and hydroquinone dissolved in water, said hydroquinone exceeding in mol percent the amount of the triaminopyridine.

20 25 No references cited.